

June 5, 1923.

R. G. OSBORNE

1,457,598

PROTECTING REINFORCEMENT IN CONCRETE AND THE LIKE

Filed Dec. 27, 1921



Inventor:  
Raymond G. Osborne

By *James D. Bullock*

his attorney

## UNITED STATES PATENT OFFICE.

RAYMOND G. OSBORNE, OF LOS ANGELES, CALIFORNIA.

PROTECTING REINFORCEMENT IN CONCRETE AND THE LIKE.

Application filed December 27, 1921. Serial No. 523,149.

*To all whom it may concern:*

Be it known that I, RAYMOND G. OSBORNE, a citizen of the United States, residing at Los Angeles, in the county of Los Angeles and State of California, have invented certain new and useful Improvements in Protecting Reenforcements in Concrete and the like, of which the following is a specification.

This invention relates to the protection of the reinforcing elements, such as reinforcing steel, in reinforced concrete, and similar bodies; and the invention provides a reinforced concrete structure wherein the reinforcing steel is more completely protected from deterioration,—the action of the elements, electrolysis, etc., than is the case in the best current practice. While reinforced concrete has been used with fairly good results under very difficult conditions, such as in the presence of sea water, in the form of concrete piles, etc., it has been found that the reinforcing steel is very apt to rust. This also is the case in all kinds of reinforced concrete structures, exposed to ordinary weather conditions; and although my invention has great advantages as applied generally to reinforced concrete or the like, its advantages are perhaps more marked as applied to such structures as concrete piles, sea walls, etc., that are subjected to the action of sea water and air and to pipe exposed to alkali action, etc.

Any rusting action, or any chemical transformation, of the reinforcing steel, is accompanied with an increase of volume, which very frequently results in cracking the enveloping concrete. Once the concrete develops cracks, the imbedded steel is more than ever exposed, and the final destruction of the concrete structure is greatly hastened.

To protect the reinforcing steel from chemical action and to prevent cracking of the enveloping concrete, several methods have been more or less commonly used. The concrete may be waterproofed by proper selection of aggregates, thus making dense mixtures, or by admixing some waterproofing or water repelling material in the concrete. Such methods as these, and also the well known method of merely superficially coating the concrete body, are aimed at protecting the steel by making the concrete body itself impervious, or as nearly impervious as may be, to water. On the other hand, it has

been more or less common to coat the steel itself in some manner, as by galvanizing or painting with waterproof paint. But all of these methods have their inherent disadvantages. It is almost impossible in practice to make any concrete that is absolutely waterproof, either by properly proportioning its constituents or by mixing the waterproofing material with it; for several reasons, among which is the impossibility in practice of obtaining an absolutely uniform mixture. Furthermore, the use of waterproofing compound mixed in concrete usually lessens the strength of the finished structure and also has a tendency to decrease the strength of bond between the concrete and steel. Waterproofing the steel itself by giving it a surface covering prior to putting it into concrete has several disadvantages; such as that bending the rods will cause the surfacing to crack or break off and also that the surfacing is apt to be locally broken or removed during the handling of the steel. And, furthermore, the painting of the steel with a protective coat usually lessens to a very great degree, if it does not destroy, the bond between the concrete and the steel; with the result that the concrete of the structure is liable to develop cracks before the proper proportion of the load is borne by the steel. My method provides for the waterproofing of reinforcing steel after it is imbedded and after the concrete has set. This, according to this invention, is accomplished by actually depositing a coat of waterproofing material on the surface of the imbedded steel after the concrete has set, or by depositing in the interstitial spaces of the concrete, around the reinforcing steel, a sufficient amount of waterproofing material to form a waterproof envelop around the steel. Such zone of waterproofing in the concrete, surrounding the steel, may be either directly adjacent the steel, or it may be further out, and nearer the exterior surface of the concrete. In any such case the steel is thoroughly protected against water and atmospheric action and is entirely protected from chemical change of all sorts.

Suppose, for instance, we take a reinforced concrete pile as an illustration and describe how its reinforcing steel may be, according to this invention, waterproofed; and describe the final quality of the resultant product. Such description will suffice to set out the whole of the invention,

as it will be then readily apparent how the invention may be applied to other structures. For this purpose a reinforced concrete pile is illustrated in the accompanying drawings, the single figure being a cross-section of a typical pile.

The reinforcing steel  $R$  having been set in the concrete  $C$  as desired, the concrete having set, and having preferably aged until it has acquired sufficient strength, then the finished body may be subjected to a process that involves substantially the heating of a porous body up to such a temperature as will expel a large proportion of the air contained in its interstitial spaces, or of the free water, or additionally, but not necessarily, a portion of the water of combination and then allowing the heated body to cool in the presence of a liquid waterproofing substance, such for instance, as heated asphalt. Upon cooling, the suction in the interstitial spaces draws the waterproofing substance through the interstitial spaces and causes them to be more or less filled. If the body is allowed to cool down to a sufficient extent, while still in the presence of the waterproofing substance, and if the body has been initially heated enough, and if its porosity, and the fluidity of the liquid are sufficient, its interstitial spaces will be completely filled with the waterproofing substance. If, however, the concrete body is removed from the presence of the waterproofing substance before it has cooled to any great extent, then the waterproofing substance that has entered the interstitial spaces will be drawn further into the body of concrete, leaving the outer interstitial spaces then more or less unfilled with the waterproofing substance. Or, by using only a moderate initial high temperature; and consequently having only a moderate amount of suction in the interstitial spaces, then of course the waterproofing substance, (for instance asphalt) will not penetrate very far below the surface of the concrete.

From these observations it will be readily understood that the radial-thickness of the layer or zone in which the interstitial spaces are filled with the water-proofing substance, can be readily controlled: as can also the position of that zone—that is, whether near or far removed from the outer surface of the concrete. I have, in the past, found that by this method here generally described I am able to cause asphalt in liquid state to penetrate throughout the body of concrete structures. Consequently I can put that interstitially filled layer or zone at any desired distance from the concrete surface, and may make it of any desired thickness.

In the case where the liquid asphalt, or other waterproofing substance, is carried

clear into the central part of the concrete, or far enough to come into contact with the exposed surfaces of the reinforcing steel, (for instance to the line  $L$ ) it will be apparent that the liquid asphalt will then come directly into contact and directly coat those portions of the steel surface that are not directly engaged by the concrete particles. In other words, the liquid asphalt, passing inwardly through the interstitial spaces, will come into contact with and coat the reinforcing steel on all those surface parts that are exposed to the interstitial spaces—on all those surface parts that could be reached under any conditions by water or air passing through the interstitial spaces. The bond of the concrete with the steel is not materially interfered with, such bond having been made and completed before the waterproofing material is introduced. That bond is caused by the innumerable concrete particles contacting with and bonding with the surface of the steel. The waterproofing material, when introduced, fills all of the interstitial spaces around the particles that make actual direct contact and bond with the steel; and therefore, without materially detracting from the direct bond of the concrete with the steel, they entirely waterproof the steel by actually coating the otherwise exposed surfaces of steel. At the same time, the adhesion of the asphalt or other waterproofing compound to the steel, and also to the surrounding concrete particles, may increase the strength of the bond between the steel and concrete.

Where all the free water has been initially expelled from the concrete, the asphalt then has a very great tendency to impregnate the concrete wholly and this is particularly true where a part of the water of combination has also been expelled. In those instances the asphalt tends to fill the voids and impregnate the cement itself: so much so that the concrete, if broken or cut open, shows completely black and the steel itself tends to be completely coated with the asphalt.

Where the asphalt is put directly against the steel as a coating, I may introduce only sufficient asphalt substantially to do nothing more than to coat the surfaces of the steel, or to fill, if any, very little depth of the surrounding concrete. But on the other hand, in practice, it will be preferred to introduce sufficient asphalt to fill the surrounding interstitial voids to at least some radial depth around the reinforcing steel; (as for instance to the line  $L'$ ); if not for any other reason, to provide a sufficient surplus of waterproofing material to be sure that every exposed surface part of the steel is covered. Or, if desired, the waterproofing material may be introduced in sufficient

quantities to fill all of the interstitial spaces further out or clear out to the exterior surface.

In a case where the reinforcing layer has not been allowed to penetrate into the concrete as deeply as the reinforcing elements, it will still be seen that the reinforcing elements are protected against external conditions, because no fluid, (water or air) can pass in through the concrete and reach the steel; all of the interstitial spaces, even the most minute in the cement itself, being filled.

I do not wish my invention, either in its aspect as process, or its aspect of finished product, to be limited specifically to the particular type of process herein explained; because the process may be carried out and the product may be produced in other manners. For instance, where it is desired to put the protective coating directly on the exposed surfaces of the reinforcing steel, that protective coating may be carried into and through the concrete and against the steel by a liquid carrier that will dry. For instance, asphalt carried by a volatile hydro-carbon may be introduced, by creation of a vacuum interiorly; and the drying out of the volatile hydrocarbon will leave the asphalt coating on the exposed surfaces of the steel. And also, as will readily be seen, substances other than asphalt may be used; such as coal-tar, pitch, paraffin, wax, etc.,—in fact any substance having the necessary qualities as herein set out. And also it will be seen that any such protective substance may be carried into the concrete by any pressure action,—that is by any means whereby the interior pressure is made lower than the exterior pressure; and this may be done by raising the exterior pressure, or lowering the interior, or both, provided always that the contained air and water are expelled from the voids. Also the protective substance in liquid form may be introduced by capillary action alone or in conjunction with

pressure, when the contained air and water have been removed.

In whatever manner the final product is produced, there results a reinforced concrete or other structure in which the reinforcing elements are completely protected, not only against the action of water and electrolysis, but also against the action of air; and one in which the strength of the concrete and the bond between the concrete and the steel are both very greatly increased. I have explained how the effectiveness of the bond is increased; and I have also found that the introduction of such waterproofing materials into the interstitial voids of the concrete greatly strengthens the concrete. And thus my product is one in which not only the reinforcing elements are thoroughly protected, but also one in which the ultimate strength of the structure is materially increased.

I claim:

1. A reinforced concrete structure wherein in the interiorly exposed surfaces of the reinforcing elements are treated with a protective substance and the interstitial spaces around the reinforcing elements are filled with such substance.

2. A reinforced concrete structure wherein the reinforcing elements are directly coated with protective substance only on their surface portions that are not actually contacted and covered by concrete particles.

3. A reinforced concrete structure wherein in the reinforcing elements are directly coated with a protective substance on their surface portions that are not actually contacted and covered by concrete particles, and wherein the interstitial spaces surrounding the reinforcing elements are filled with protective substance.

In witness that I claim the foregoing I have hereunto subscribed my name this 15th day of December, 1921.

RAYMOND G. OSBORNE.